

## UNITED STATES PATENT OFFICE.

ALBERT L. CLAPP, OF DANVERS, MASSACHUSETTS, ASSIGNOR TO THE FLINTKOTE COMPANY, OF BOSTON, MASSACHUSETTS, A CORPORATION OF MASSACHUSETTS.

## SHINGLE MATERIAL AND METHOD OF MANUFACTURE.

No Drawing.

Application filed September 12, 1923. Serial No. 662,225.

This invention relates to prepared shingles and a method of manufacturing the same, the object of the invention being to produce a waterproof shingle having the property of 5 remaining flat under all weather conditions, and which may be completely formed on a paper machine, without subsequent saturating or coating processes.

Much trouble has been experienced with 10 shingles formed of the so-called asphalt roofing, which is commonly composed of rag felt saturated with asphalt and then provided with a suitable surface layer such as a coating of high melting point or blown asphalt, and 15 an exposed facing of granular material such as crushed slate thereto, due to the curling or warping of the shingles after they have been laid in position on the roof. Heretofore it has generally been believed that this curling 20 and warping is due to faulty saturation of the material permitting exposure of the fibers to the weather to absorb and give off moisture with changing atmospheric conditions. Much attention has therefore been directed 25 to the problem of insuring as complete saturation as possible in order to seal the fibers against exposure to the atmosphere. From considerable experimentation I have come to the conclusion that imperfect saturation 30 plays only a minor part in such warping and curling. Irrespective of the amount of saturant commercially employed in such material, I have found that it readily absorbs from 6% to 50% by weight of moisture when immersed 35 in water for twenty-four hours. This does not necessarily mean that the material is not water resistant, but merely that it is practically impossible to prevent capillary absorption of water into the cells of the individual fibers irrespective of the thoroughness 40 with which the felt is saturated with waterproofing material.

It is my belief that the cause of the curling and warping is chemical change within the 45 more or less hydrated individual fiber cells, the hydrated cellulose being unstable, the amount of water within the fibers occurring either as chemically combined with the cellulose or free and being variable under variable climatic conditions.

I have found that certain fibers have less tendency to hydrate and to absorb water than others, and that the fibers which have great capacity for hydration and absorption of

water by the capillary cells also show a strong 55 tendency for the felted material made therefrom to warp and curl, when dry, under changes in atmospheric conditions. Arranged in their order as to their capacity of hydration and cellular capillary absorption, the 60 various cellulosic fibers in common use may be listed somewhat as follows: (1) rope and sulphate pulp, (2) sulphide pulp, (3) "news" pulp and (4) rags. That is, a board made from sulphate pulp or rope after being dried 65 curls more than one made from sulphite pulp beaten out the same length of time, and a board made of sulphite pulp curls more than one made of "news" pulp or of rags beaten out the same length of time. It should be 70 noted, however, that there is considerable danger of curling even with the more inert cellulose fibers such as those of rags, in case they are beaten out hard for a considerable 75 length of time so as to become hydrated. I have found that old rags have less capability of hydration and cellular capillary absorption 80 than new rags. This fact I believe to be due to the greater proportion of oxyhydrocellulose in the old rags, the presence of the oxyhydrocellulose indicating that the fibrous structure is more or less broken down, so that the capillaries of the individual fibers are less pronounced than in the new rags. This 85 condition is doubtless due to a partial oxidation of the fibers which had become more or less hydrated from exposure to atmospheric conditions. As a result of my experiments, I have found therefore that fibers which are capable of being incorporated with felted 90 material, but which are inert from chemical combination with water so as to be hydrated are free from such warping and curling tendencies. For example, asbestos fiber which is inert in respect of hydration, has a freedom from any tendency to curl and warp. 95 Asbestos fiber alone, however, does not form and felt readily on the paper machine and it is therefore desirable, in order to produce proper felting, to mix it with other fibers, such for example as rags, which in themselves are the freest of the various cellulose materials from curling and warping tendencies.

Smaller proportions of "news", still smaller proportions of sulphite and yet smaller proportions of sulphate pulp may also be used without permitting the curling and warping 100 tendencies of these latter fibers to overcome 105

the inert nature of the asbestos fibers so as to cause the final product to curl or warp. When exposed to the weather for a long period of time the cellulose fibers of the ordinary asphalt shingles such as are commonly made from rag felt saturated and coated with asphalt, becomes oxyhydrated but by that time the asphalt itself has become oxidized and brittle. The oxyhydration of the cellulose fibers destroys the strength of the shingle and the useful life of the shingle is thus ended. The asbestos is not subject to this deterioration and thus prolongs the useful life of the shingle, especially since felted asbestos becomes denser with lapse of time.

I propose, therefore, to employ asbestos fiber or other non-hydratable fiber as the major or preponderant portion of the fibrous material to be used, together with sufficient cellulose materials, preferably of the least possible hydrating tendencies and beaten as little as possible, to form a fibrous mixture capable of being run off satisfactorily on the paper machine and, which, when dried, has little or no tendency to curl. Also in order to avoid the necessity of saturating the material so formed in order to render it waterproof, I propose to incorporate the waterproofing material in the fibrous pulpy stock so that the sheet as initially formed contains the waterproofing agent. It might also be stated here that it is difficult to saturate felted asbestos. Any desirable coloring matter may also be incorporated to give the desirable color to the finished material.

For example, one may proceed as follows: 30 parts of asbestos (long or short fiber), 15 parts of rags, 15 parts of newspaper and a sufficient quantity of water are loaded into a beater together with any suitable coloring matter (which, if desired, may comprise one part Prussian blue) 2 parts red iron oxide, 2 parts ivory black, and 1 part nigrosine; and powdered unsaponified waterproofing materials, such as 20 parts of montan wax and 20 parts of gilsonite, and the mixture is hard beaten for 2 hours. 5 parts of rosin size and 5 parts of silicate of soda are then added and mixed in for 20 minutes, whereupon 10 parts of aluminum sulphate or other suitable precipitant are then added and beaten in for 20 minutes to precipitate the size and silicate of soda in the form of a coagulum which fixes the unsaponified waterproofing materials, i. e., the wax, gilsonite, and coloring matter on the fibers. This pulp is then transferred to any suitable paper making machine, e. g. a wet paper machine and when of the desired caliper the sheet removed therefrom in the form of a board. This board is then air dried, the discrete or finely divided particles of thermo-plastic material fluxed and coalesced by heat and pressure, calendered and cut into shingles.

65 I have found that asbestos is most desirable

fiber to prevent the shingles from curling or warping but that any proportion of sulphate pulp above about 30% causes curling and warping even though asbestos is used. The curling properties of cellulosic fibers, for example sulphate pulp, may be overcome to some extent by the use of sawdust (e. g. 40 mesh) or wood flour, which lack a fibrous structure. It is also possible to employ wood flour in considerable quantities with the asbestos thereby reducing the quantity of cellulosic fiber to be employed, the wood flour acting to hold the asbestos fibers together so that they may be formed and felted. This causes the completed board to be less porous, and aids in holding the waterproofing materials incorporated in the pulp while it is being run on the paper machine. For example, 10% asbestos, 30% of wood flour and 10% of rags by weight may be successfully used in the pulp.

In place of the montan wax and gilsonite as stated in the example hereinbefore given, one hundred parts of (wet) asphalt emulsion made according to the Kirchbraun method and 20 parts of powdered montan wax or gilsonite may be used. This asphalt emulsion is made by emulsifying or dispersing a normally adhesive asphalt in water with a colloidal clay emulsifying agent, and is known to the trade as "K-B emulsion". For example, the furnish may consist of 50 parts asbestos, 10 parts rag, 20 parts montan wax, 100 parts of wet K-B emulsion, 1 part ivory black, 5 parts rosin size, 10 parts silicate of soda, and 20 parts aluminum sulphate. The emulsion alone is too flabby to serve as the entire waterproofing material of a rigid shingle, but by the addition of a hard thermoplastic material such as montan wax or gilsonite, the product is rendered quite stiff and rigid. A suitable shingle, however, may be produced by the use of K-B emulsion alone as the waterproofing agent. Together with the various waterproofing agents above enumerated, leather dissolved in caustic soda may be used. For example, the furnish may comprise 50 parts of asbestos, 30 parts of rags, 100 parts wet "K-B emulsion", 20 parts of leather, 2 parts of caustic soda, and 8 to 10 parts of alum. The asbestos and rags are beaten up together, and the leather and caustic may be mixed together with water to form a leather solution, which may be added to the beater, or the leather and caustic may be added separately to the beater and the solution of the leather effected therein. After the leather solution has been thoroughly mixed with the fibers, the K-B emulsion is incorporated in the pulp and then the alum is added. This precipitates the leather in insoluble gelatinous form which fixes the waterproofing agent on the fibers. The stock is then run off on the paper machine and further treated as hereinbefore described.

The precipitated leather forms a more or less waterproofing agent which is not subject to deterioration by oxidation on exposure to the weather. Of course any desired coloring matter may be added to the furnish to color the final product.

Adverting once more to the use of various forms of fibers which may be employed in the manufacture of so-called asphalt shingles, 10 it is my belief that when cellulose fibers are hydrated, more or less, in the preparation of the pulp, the fibers, even after the sheet is dried as ordinarily, contain water of hydration, which is alternately freed and again 15 chemically combined with the cellulose cells, under the conditions to which such shingles are subjected in use. These chemical changes result in physical changes in the shingle, which are manifested by the curling and 20 warping thereof, this taking place in spite of the coating or surfacing materials with which such shingles are ordinarily provided. Consequently when cellulosic fibers are 25 pulped with inert fibers, such as asbestos, the beating operation should be so carried on as to effect a homogeneous mixture with the least possible hydration of the cellulose fibers. A sheet formed solely of asbestos does not 30 expand and contract when exposed to the weather for an indefinite period of time and neither curls nor warps, but lies flat. Consequently for the best results only that proportion of cellulosic material should be 35 mixed with the asbestos in the pulping operation, as is necessary for the proper formation and felting of the finished sheet. The examples hereinbefore given of various proportions of the components are intended to 40 serve only as guides in the practice of my invention, as of course the proportions and the particular ingredients may be changed, provided the principles herein pointed out are borne in mind. It might also be noted that 45 when the non-hydrating fiber used is asbestos the shingle is rendered quite fireproof.

While the term "shingle" has been herein used it should be understood that this is intended to include shingles, shingle strips and other individual weather-proofing elements 50 formed from sheet material.

Having thus described this invention it will be evident to those skilled in the art that many modifications and changes might be made without departing from its spirit or 55 scope as defined by the appended claims.

I claim:

1. The method of forming a shingle which comprises beating up asbestos fiber, cellulosic fiber and waterproofing material in water, 60 then adding precipitable sizing and continuing the beating, then adding a precipitant for the sizing and beating, running off on a paper machine, and then fluxing, and finally cutting the sheet thus formed into 65 roofing shingles.

2. The method of forming a shingle which comprises beating up asbestos fiber, cellulosic fiber, comminuted cellulosic material, and waterproofing material in water, then adding precipitable sizing and continuing the 70 beating, then adding a precipitant for the sizing and beating, running off on a wet paper machine, and then fluxing and calendering, and finally cutting the sheet thus formed into roofing shingles. 75

3. The method of forming a shingle which comprises beating up asbestos fiber, cellulose fiber and waterproofing material in water, then adding precipitable sizing and continuing the beating, then adding a precipitant 80 for the sizing and beating, running off on a wet paper machine, and then air drying, fluxing and calendering, and finally cutting the sheet thus formed into roofing shingles.

4. A shingle comprising a fibrous foundation having the felted characteristics of paper machine fabrication and comprising asbestos, and bituminous waterproofing material coalesced throughout said foundation. 85

5. A shingle comprising a fibrous foundation having the felted characteristics of paper machine fabrication and consisting of asbestos and cellulosic material, and bituminous waterproofing material coalesced 90 throughout said foundation. 95

6. A shingle comprising a fibrous foundation having the felted characteristics of paper machine fabrication and consisting of asbestos and cellulosic material, the asbestos forming the major portion of said foundation, and bituminous waterproofing material 100 coalesced throughout said foundation.

7. A shingle comprising a fibrous foundation having the felted characteristics of paper machine fabrication and comprising non-hydrating fibrous material, a waterproofing agent, and a waterproofing coagulum permeating said foundation. 105

8. A shingle comprising a fibrous foundation having the felted characteristics of paper machine fabrication and comprising non-hydrating fibrous material, and a thermo-plastic waterproofing agent and coloring matter permeating said foundation. 110

9. A shingle comprising a fibrous foundation having the felted characteristics of paper machine fabrication and comprising non-hydrating fibrous material, and a thermo-plastic waterproofing agent and coloring matter permeating said foundation and fixed to the 115 fibers. 120

10. A shingle comprising a fibrous foundation of cellulosic material and asbestos having the felted characteristics of paper machine fabrication, said foundation having hard wax, asphalt emulsion, coloring matter, and a waterproofing coagulum permeating the foundation and fixed to the fibers thereof. 125

11. A shingle comprising a fibrous foundation of cellulosic material and asbestos 130

having the felted characteristics of paper machine fabrication, said foundation having asphalt emulsion, coloring matter, and a waterproofing coagulum permeating the 5 foundation and fixed to the fibers thereof.

12. Sheet material comprising a fibrous base containing a preponderating proportion of non-hydrating fiber and having the felted characteristics of paper machine fabrication, 10 and a waterproofing material fixed on said fiber with a coagulum.

13. Sheet material comprising cellulosic material, asbestos, and precipitated leather.

14. A non-warping, non-curling roofing 15 material consisting of a sheet of fibers, felted on a paper making machine, said fibers comprising a preponderating proportion of fibers inert to hydration, together with sufficient cellulosic fibers to permit the felting of 20 the fibrous mass on a papermaking machine, and containing a thermo-plastic waterproof-

ing compound coalesced in the sheet from finely divided particles thereof.

15. A shingle comprising a fibrous foundation of cellulosic and asbestos fiber filled 25 with comminuted cellulosic material and felted on a papermaking machine, said foundation being permeated with unsaponified thermoplastic waterproofing material fixed to said fiber by precipitated waterproofing material. 30

16. A shingle comprising a fibrous foundation of cellulosic asbestos fiber, filled with comminuted cellulosic material and felted on a papermaking machine, said foundation being permeated with the coalesced particles 35 of finely divided asphalt and hard wax fixed to said fiber by precipitated leather.

In testimony whereof I have affixed my signature.

ALBERT L. CLAPP.